

[54] PREPARATION OF POLYMERIC  
REACTION PRODUCTS OF  
ALKOXYALKYLAMINES AND  
EPIHALOHYDRINS[75] Inventors: Gary W. Y. Kwong, Racine, Wis.;  
Joseph Levy, Deerfield Beach, Fla.

[73] Assignee: UOP Inc., Des Plaines, Ill.

[21] Appl. No.: 197,033

[22] Filed: Oct. 15, 1980

## Related U.S. Application Data

[63] Continuation-in-part of Ser. No. 92,384, Nov. 8, 1979,  
Pat. No. 4,252,745.[51] Int. Cl.<sup>3</sup> ..... C07C 85/04; C07C 89/02

[52] U.S. Cl. ..... 564/476; 564/477

[58] Field of Search ..... 564/476, 477, 475

## [56] References Cited

## U.S. PATENT DOCUMENTS

1,790,042 1/1931 Eisleb ..... 564/476 X

|           |         |                       |           |
|-----------|---------|-----------------------|-----------|
| 3,257,250 | 6/1966  | Perry et al. ....     | 564/476 X |
| 3,424,681 | 1/1969  | Stanford ....         | 564/483 X |
| 3,499,930 | 3/1970  | Wakeman et al. ....   | 564/297   |
| 3,567,659 | 3/1971  | Nagy ....             | 564/476 X |
| 3,636,114 | 1/1972  | Tobler et al. ....    | 564/292   |
| 3,855,158 | 12/1974 | Petrovich et al. .... | 564/476 X |
| 3,855,299 | 12/1974 | Witt ....             | 564/476   |
| 4,140,798 | 2/1979  | Merianos et al. ....  | 564/476 X |
| 4,178,434 | 12/1979 | Langdon ....          | 564/505 X |

Primary Examiner—John Doll

Attorney, Agent, or Firm—James R. Hoatson, Jr.;  
Eugene I. Snyder; William H. Page, II

## [57] ABSTRACT

A process for preparing novel polymeric reaction products comprises commingling one molar proportion of an alkoxyalkylamine with from about 0.5 to about 2.0 molar proportions of an epihalohydrin at a temperature from about 40° C. to about 150° C. in the presence of an inorganic base, and recovering the reaction products. Epichlorohydrin is a preferred epihalohydrin.

8 Claims, No Drawings

PREPARATION OF POLYMERIC REACTION  
PRODUCTS OF ALKOXYALKYLAMINES AND  
EPIHALOHYDRINS

CROSS-REFERENCE TO RELATED  
APPLICATION

This application is a continuation-in-part of our co-pending application, Ser. No. 92,384, filed Nov. 8, 1979 now U.S. Pat. No. 4,252,745, all of which is incorporated herein by reference.

BACKGROUND OF THE INVENTION

Various types of petroleum-derived hydrocarbon oil undergo deterioration on storage or upon exposure to severe conditions. Thus fuel oils such as gasoline, diesel fuel, jet fuel, other aviation fuel, burner oil, furnace oil, kerosene, and naphtha, for example, and other oils such as lubricating oils, cutting oils, slushing oils, etc., undergo deterioration as evidenced by such changes as, for example, formation of sediment and discoloration.

Sediment formation is undesirable for various reasons. The settling of accumulated particulates in tanks storing hydrocarbon oils require periodic draining and cleaning of storage tanks, leading to temporary unavailability of storage capacity, substantial diversion of manpower, and waste disposal problems. Sediment formation in burner oil tends to plug strainers, burner tips, injectors, etc. In diesel fuel such sediment tends to form sludge and varnish in the engine. If the oil is used as a heat exchange medium, as for example with jet fuel, the sediment tends to plug exchanger coils. In gasoline the sediment may tend to deposit on sensitive parts in an internal combustion engine, such as carburetors, thereby decreasing the efficiency of combustion and causing increased fuel consumption.

It is apparent, therefore, that reduced sediment formation in hydrocarbon oils is desirable. One method of effecting such reduction would be to eliminate, to a substantial degree, those processes leading to particulate formation, such as oxidation. Another method would be to prevent agglomeration and/or settling of the formed particulate matter by effectively maintaining the fine particulates in a well dispersed state, for when the particulates are so dispersed the aforementioned difficulties associated with sediment formation either do not occur or are of substantially lessened severity.

Discoloration of hydrocarbon oils is undesirable because it is an indication that degradation has occurred or is occurring, hence there is a marked customer preference for lighter oils. Thus there is an economic incentive for minimizing discoloration and degradation of hydrocarbon oils, especially during long-term storage.

SUMMARY OF THE INVENTION

This invention relates to the preparation of a novel reaction product. One embodiment comprises commingling 1 molar proportion of an alkoxyalkylamine, wherein the alkoxy group contains from about 1 to about 25 carbon atoms, the alkyl group is an alkylene group containing from 2 to about 10 carbon atoms, and the amine is a primary amine which may contain multiple alkylene amino units, with from about 0.5 to about 2.0 molar proportions of an epihalohydrin, at a temperature from about 40° C. to about 150° C. in the presence of an inorganic base. In a more specific embodiment said epihalohydrin is epichlorohydrin. In a still more

specific embodiment said alkoxy group contains from about 6 to about 20 carbon atoms, said alkyl group is a propylene group, said amine moiety is  $-\text{NH}_2$  or  $-\text{NH}(\text{CH}_2)_3\text{NH}_2$ , and said epihalohydrin is epichlorohydrin.

DESCRIPTION OF THE INVENTION

The compositions of matter prepared according to the process of this invention are polymeric reaction products of an alkoxyalkylamine with an epihalohydrin formed at a reaction temperature from about 40° C. to about 150° C. in the presence of an inorganic base. Such reaction products have a broad range of uses, as is described within. Additionally, such reaction products generally have relatively low pour points and viscosities. Such attributes are desirable in ease of handling and utilizing these materials in their perceived uses. For example, additives for hydrocarbon oils frequently are metered into the oil by pumping under a wide range of temperatures, and it is desirable that such additives remain liquid and pourable, with not too high a viscosity at low temperatures, to ensure pumpability.

As mentioned previously, the materials of this invention are polymeric reaction products of an alkoxyalkylamine with an epihalohydrin under the aforementioned reaction conditions. The reaction frequently is conducted in a high-boiling, unreactive solvent to moderate the exothermic reaction and for ease of manipulation, both during the reaction and afterwards. However, the use of a solvent, where such use is undesirable, may be eliminated although the results may not be necessarily equivalent. Among the solvents which may be used are included toluene, xylene, mesitylene, ethylbenzene, propylbenzene, and other alkylated and polyalkylated aromatics as examples of suitable high-boiling but unreactive materials.

The term "alkoxyalkylamines" as set forth in the specification and appended claims will include primary amines and will include monoamines, diamines, triamines, etc. Where monoamines are used the amine can be represented as  $\text{ROR}_1\text{NH}_2$ . The alkoxy group,  $\text{RO}$ , of such monoamines contains from about 1 to about 25 carbon atoms, but preferably from about 6 to about 20 carbon atoms. Suitable groups representative of the carbonaceous portion of the alkoxy group include methyl, ethyl, propyl, butyl, pentyl, hexyl, heptyl, octyl, nonyl, decyl, undecyl, dodecyl, tridecyl, tetradecyl, pentadecyl, hexadecyl, heptadecyl, octadecyl, nonadecyl, eicosyl, heneicosyl, docosyl, tricosyl, tetracosyl and pentacosyl moieties. Such groups commonly have their commercial origin in fatty acids and petroleum-derived alcohols, and consequently are often supplied as mixtures. Therefore it is to be understood that amines containing a combination of the aforementioned groups are explicitly within the scope of this invention.

When the carbonaceous portion of the alkoxy group is derived from fatty acids the major portion is an unbranched aliphatic group. When the carbonaceous portion comes from petroleum-derived olefins, the major portion generally is a branched aliphatic group. In each case minor amounts of unsaturated material may be present. Therefore it is to be understood explicitly that the carbonaceous portion of the alkoxy group of the alkoxyalkylamines of this invention may be comprised of either a major portion of unbranched or branched aliphatic groups which may contain minor amounts of unsaturation.

The alkyl group,  $R_1$ , of the alkoxyalkylamines of this invention is an alkylene group containing from 2 to about 10 carbon atoms. Examples of alkylene groups which are suitable include ethylene, propylene, butylene, amylene, hexylene, heptylene, octylene, nonylene, and decylene. In a preferred embodiment the alkylene group is propylene. Such alkylene groups generally are unsubstituted, but branched alkylene groups may be employed, not necessarily with equivalent results. Examples of the latter include isopropylene, sec-butylene, iso-butylene, sec-amylene, iso-amylene, etc.

It is a discovery of this invention that diamines, triamines, tetramines, etc., also form polymeric reaction products of this invention. In the case of diamines the structure may be represented as  $R-O-R_1NHR_2NH_2$ , where  $RO$  and  $R_1$  bear the same description as that set forth above for the monoamines. The group  $R_2$  is, like  $R_1$ , an alkylene group containing from 2 to about 10 carbon atoms, generally unbranched but not necessarily so.  $R_1$  and  $R_2$  may be the same or may be different. Examples of diamines, cited solely for illustrative purposes, include alkoxyalkyl ethylenediamine, alkoxyalkyl propylenediamine, alkoxyalkyl butylenediamine, alkoxyalkyl amylenediamine, alkoxyalkyl hexylenediamine, etc., alkoxyalkyl isopropylenediamine, alkoxyalkyl isobutylenediamine, alkoxyalkyl sec-butylenediamine, and so forth. In a preferred embodiment both  $R_1$  and  $R_2$  are propylene groups,  $-CH_2CH_2CH_2-$ .

In a like manner the triamines can be represented as  $ROR_1NHR_2NHR_3NH_2$ , the tetramines as  $ROR_1NHR_2NHR_3NHR_4NH_2$ , the pentamines as  $ROR_1NHR_2NHR_3NHR_4NHR_5NH_2$ , etc., with a general formula of  $ROR_1(NHR_2)_mNH_2$ , where  $m$  is the number of secondary amino groups present in the polyamine and is an integer less than about 10. The description of  $RO$  and  $R_1$  in such polyamines conforms to that given hereinbefore. In the embodiment where  $m$  is equal to or greater than 2, the group  $R_2$  is an alkylene group otherwise conforming to the description hereinbefore set forth for  $R_1$ . Examples of such amines include alkoxyalkyl diethylenetriamine, alkoxyalkyl triethylenetetramine, alkoxyalkyl polyethyleneimine, alkoxyalkyl dipropylenetriamine, etc.

Just as the alkoxy group may contain a combination of carbonaceous groupings, so may the diamines, triamines, etc. contain a combination of polyamines. Therefore it is to be understood that this invention encompasses all mixtures of amines whose major components conform to those descriptions set forth above.

The amine or mixture of amines is reacted with an epihalohydrin. Epichlorohydrin is preferred, although epibromohydrin and epiodohydrin may be used but not necessarily with equivalent results in every case. Other epihalohydrins which may be employed in this invention include 1-chloro-3,4-epoxybutane, 1-chloro-2,3-epoxybutane, 1-chloro-4,5-epoxypentane, 1-chloro-3,4-epoxypentane, etc., and the corresponding bromo and iodo compounds. Suitable condensation products may also be obtained when using a mixture of epihalohydrins, where each of the components meets the qualifications set forth above. The amount of epihalohydrin used ranges from about 0.5 to about 2 moles per mole of amine. Preferably the molar ratio of epihalohydrin to alkoxyalkylamine is in the range from about 0.7 to about 1.2.

The process of this invention is effected by contacting the epihalohydrin and amine, generally in a high boiling aromatic solvent, at a suitable temperature, and

removing the inorganic halide which forms with an inorganic base. Generally the reaction may be conducted at a temperature from about 40° C. to about 150° C., a preferred temperature range being from about 60° C. to about 125° C. Inorganic bases suitable for use in the present invention include the alkali metal hydroxides and carbonates, and the alkaline earth oxides, hydroxides, and carbonates. Examples of such materials, cited for illustrative purposes only, are the hydroxides and carbonates of lithium, sodium, potassium, rubidium and cesium, magnesium oxide, magnesium hydroxide, magnesium carbonate, calcium oxide, calcium hydroxide, calcium carbonate, barium oxide, barium hydroxide, and barium carbonate. Where the epihalohydrin is used in up to equal molar proportions of the amine, then the molar amount of base employed is approximately equal to that of the amine, although an excess of base over amine up to about 50% often may be employed advantageously. Where the epihalohydrin is used in greater than molar proportions relative to amine, then the molar amount of base is about equal to that of epihalohydrin although an excess up to about 50% may be used.

The mode of preparation of this invention is susceptible to numerous variations on the theme of directly reacting the amine with the epihalohydrin under reaction conditions. An example of one general mode is the addition of epihalohydrin to a solution of the amine in a suitable solvent, generally a high-boiling aromatic compound or mixtures thereof. Reaction between the components occurs to a given acidity, or given amount of amine hydrohalide formation, at which time either aqueous or solid inorganic base is added to remove the halide thus formed. The primary reaction product therefrom undergoes further condensation leading to the ultimate reaction product.

An example of another mode of preparation is the concurrent addition of epihalohydrin and amine to the solvent employed at a suitable temperature. When reaction has occurred to a desired amount of acidity, aqueous or solid inorganic base is added and the liberated primary reaction product thereupon undergoes further condensation leading to the ultimate reaction product.

In still another method of preparation, the epihalohydrin and amine are added concurrently to the solvent containing a portion of the inorganic base employed. The base may be either in solution or as a solid. After reaction has occurred to a given amount of acidity the remaining portion of solid or aqueous base is added and the primary reaction product thereupon undergoes further condensation leading to the ultimate reaction product.

The materials formed in the process of this invention have been shown to be good dispersants of particulates while being poor dispersants of water. This combination of properties is an excellent one for use of these materials as sedimentation inhibitors of hydrocarbon oils, especially fuel oils. Additionally, the materials described herein show substantial inhibition of discoloration in hydrocarbon oils. Thus these materials are superior additives for preserving quality of hydrocarbon oils upon storage, especially at elevated temperatures or for relatively long periods of time. The polymeric reaction products of this invention may also be anticipated

to have significant potential as corrosion inhibitors, carburetor detergents, antifoulants, lubricant additives, etc.

The following examples are merely illustrative of this invention, and it is to be understood that the invention is not necessarily limited thereby.

#### EXAMPLE I

Epichlorohydrin (83.2 g, 0.90 mol) was added dropwise over about 50 minutes to a stirred, pale yellow solution, initially at about 90° C. of tridecyloxypropylamine (280.4 g, 1.05 mole), dissolved in 222 g. of Espesol 3BC. The latter is the trade name for high boiling bottoms from xylene fractionation as supplied by Charter Oil Co. The solution was stirred about 1.5 hours at 94°-110° C., after which a solution of 20% aqueous sodium hydroxide containing 0.99 mole of base was added over about 40 minutes while the reaction temperature was maintained at 86°-94° C. The mixture was stirred about 2.5 hours at 86°-91° C., and an additional 0.09 mole of base in water was added. The mixture was cooled, layers were separated, and the organic phase was filtered to give a clear, amber solution (544 g) which contained 53.2% active ingredient by the nitrogen jet gum method, ANSI/ASTM D381-70 modified in that nitrogen is used as the gas.

#### EXAMPLE 2

Epichlorohydrin (0.240 mol) was added over 50 minutes to a pale yellow solution of N-tridecyloxypropyl-1,3-propylenediamine (0.26 mol) in 60 g. of the aforementioned solvent at 76°-80° C. The mixture was stirred at 77°-83° C. for about 30 minutes, and 0.26 mole of a 20% aqueous sodium hydroxide solution was added over 15 minutes. Stirring at 78°-83° C. was continued about 1.8 hours, an additional 0.024 mole of base was added, and the mixture was stirred an additional 0.5 hr. at 82°-83° C. Finally layers were separated, 10 g. xylene was added to the organic phase, and water was removed by azeotropic distillation to give 152 g. (96%) of a clear yellow solution containing 54% of active ingredient.

#### EXAMPLE 3

Tridecyloxypropylamine (0.750 mol) and epichlorohydrin (0.712 mol) were added separately but concurrently to a stirred mixture of Espesol 3BC (160 g.) and 22% aqueous sodium hydroxide containing 0.0712 mole base at 73°-83° C. over a period of 1.5 hr. After an additional 10 min. at 80° C. 22% aqueous sodium hydroxide containing 0.712 mole of base was added over 13 min. The mixture was stirred at 78°-87° C. for 1 hour, then at 110° C. for 2 hr. Layers were separated and the organic phase was filtered to give 387 g. (97%) of a solution containing 53.4% of active ingredient.

#### EXAMPLE 4

N-Tridecyloxypropyl-1,3-propylenediamine (0.740 mol) and epichlorohydrin (0.70 mols) were added concurrently over about 40 minutes to mixture of Espesol 3BC (172 g.) and 22% aqueous sodium hydroxide containing 0.070 mole of base at 75°-90° C. After 8 minutes additional 22% aqueous sodium hydroxide (0.70 mole of

base) was added over 15 min. The temperature was increased to 110° C. over 1 hour and the mixture was stirred for 2 additional hours at that temperature. Layers were separated, 15 g. of xylene was added to the organic phase, and water was removed by azeotropic distillation to give 423 g. (97%) of a light amber solution containing 53% of active ingredient.

#### EXAMPLE 5

An alkoxypropyl-1,3-propylenediamine mixture rich in C<sub>12</sub>-C<sub>15</sub> groupings (0.594 mol) and epichlorohydrin (0.56 mol) was added concurrently over a period of 1 hour to a mixture of 137 g. Espesol 3BC and 22% aqueous sodium hydroxide (0.056 mol) at 71°-91° C. After 5 minutes, 0.56 mole of additional base, as a 22% aqueous solution was added with stirring at 83°-92° C. over 13 min. The temperature was raised to 108° C. and the mixture was stirred at 106°-9° C. for about 3½ hour. Layers were separated, 15 g. xylene was added to the organic phase and water was removed by azeotropic distillation to give 361 g. (96%) of a clear yellow solution containing 54.3% active ingredient.

We claim as our invention:

1. The process of making a polymeric reaction product which comprises reacting one molar proportion of an alkoxyalkylamine with from about 0.5 to about 2.0 molar proportions of an epihalohydrin selected from the group consisting of epichlorohydrin, 1-halo-3,4-epoxybutane, 1-halo-2,3-epoxybutane, 1-halo-4,5-epoxypentane, and 1-halo-3,4-epoxypentane, at a temperature from about 40° C. to about 150° C., thereafter reacting the resultant adduct with an inorganic base at said temperature, and recovering the polymeric reaction product.
2. The process of claim 1 wherein the alkoxy moiety of said alkoxyalkylamine is selected from the group consisting of aliphatic moieties containing from about 1 to about 25 carbon atoms, the alkyl moiety of said alkoxyalkylamine is an alkylene moiety containing about 2 to about 10 carbon atoms, and the amine is a primary amine selected from the group consisting of amino and (HNR<sub>2</sub>)<sub>m</sub>NH<sub>2</sub>, where m is an integer from 1 to about 10 and R<sub>2</sub> is an alkylene moiety containing from 2 to about 10 carbon atoms.
3. The process of claim 2 wherein said alkoxyalkylamine is an alkoxypropylamine.
4. The process of claim 2 wherein said alkoxyalkylamine is an alkoxypropyl-1,3-propylenediamine.
5. The process of claim 2 wherein said inorganic base is selected from the group consisting of the hydroxides and carbonates of lithium, sodium, potassium, rubidium, caesium, calcium, magnesium, and barium.
6. The process of claim 1 wherein said molar proportions of epihalohydrin are from about 0.7 to about 1.2.
7. The process of claim 1 wherein the temperature is from about 60° C. to about 120° C.
8. The process of claim 1 wherein the epihalohydrin is epichlorohydrin.

\* \* \* \* \*